

# UNITED STATES PATENT OFFICE.

EDWD. HUNT AND HENRY D. POCHIN, OF SALFORD, ENGLAND.

## IMPROVEMENT IN PREPARATION OF RESINS.

Specification forming part of Letters Patent No. 22,558, dated January 11, 1859.

*To all whom it may concern:*

Be it known that we, EDWARD HUNT and HENRY DAVIS POCHIN, both of Salford, in the county of Lancaster and Kingdom of Great Britain, chemists, have invented Improvements in the Treatment and Application of Resins and Resinous Substances; and we do hereby declare that the following is a full and exact description thereof.

Our invention or discovery consists in certain new articles of commerce produced from resin and resinous substances, and purified, clarified, and partially deprived of their color by an improved process.

To enable others to produce these new articles of commerce or secure the results we have obtained, we proceed to describe the process as conducted in three different modes, according to the nature of the apparatus employed.

In each apparatus there is a still which receives the substances to be purified, and one or more receivers communicating by a pipe or pipes with the said still. A steam-pipe, in connection with a boiler, is introduced into and reaches to the bottom of the said still, where it radiates into various smaller pipes, perforated so as to allow of the exit of steam. The size of the said steam-pipe for a still capable of holding six and a half tons of resin should, when the steam hereinafter mentioned is to be used at a pressure of ten pounds, be of the diameter of two inches.

The exact proportions and disposition of the several apparatuses, as herein described, is not material to the successful performance of the said invention; but it is material that the volume of steam should be about that which would be introduced under the conditions hereinbefore mentioned.

In the first mode of arrangement (apparatus number one) one receiver only is used, and the communication between the receiver and the still consists of a single pipe of ordinary construction. In the second mode (apparatus number two) several receivers are employed, the communication being direct from the still to one only of the said receivers, and the communication being continued by pipes from one receiver to the other. The third mode (apparatus number three) is that in which two receivers are employed, the communication of both with the said still being direct and the

pipes uniting and entering the said still as one at a point distant from the said still about three feet. These pipes are at their point of union directly one above the other.

The process as conducted with apparatus number one is as follows: The substance to be operated upon is broken into convenient lumps and thrown into the still. The still is then fired until the substance melts, when steam at the pressure hereinbefore mentioned is turned into the steam-pipe, and, passing through the perforated pipes above mentioned, thoroughly permeates the entire contents of the said still. The still is meanwhile continuously fired until the temperature of the said still rises to about 600° Fahrenheit, at which it is maintained until all such portions of the contents of the said still as are capable of being volatilized have passed from it into the receiver. The volatilization commences at a temperature of about 390° Fahrenheit. The intromission of steam is continued during the entire period of the operation. The residuum in the still consists principally of the foreign matters present in the substances before they were operated upon. The receiver is in this arrangement kept as cold as it can be by the application of water or other means, so as effectually to condense the whole of the volatile matter which has passed out of the said still during the operation. The contents of the said receiver will, on cooling, be found to consist of a certain amount of fluid and a certain amount of solid. The former (principally water condensed from the steam used in the process) is drawn off. The latter is found to present the characteristics of rosin, or other of the resinous substances operated upon, as found in its purest state. It is, however, at this stage still opaque, from containing a considerable amount of moisture. Various modes may be adopted with effect to receive the moisture from the said solid, among others that of placing it within a vacuum-pan and heating it in the usual way, or placing it within a leaden vessel surrounded by a jacket through which steam is passed, or melting it in an open leaden vessel by means of steam and passing superheated steam through it when melted.

In the process as conducted with apparatus number two, the receiver nearest to the still, and in the case of more than two receivers being em-

ployed, every receiver, except that farthest from the still, is maintained at a temperature a little above 212° Fahrenheit. The contents of the receivers nearest to the still are found to be transparent and almost free from moisture. The rosin and resinous matters condensed in the last receiver in the processes conducted by this apparatus alone contain any moisture which it is necessary to remove. This moisture may be removed in precisely the same manner as that indicated in the process hereinbefore described with reference to apparatus number one.

In the process as conducted with apparatus number three the volatile matter arising from the substances placed in the said still, as hereinbefore mentioned, arranges itself in two streams, the upper one, composed principally of steam, passing to receiver number one, and the lower one, consisting principally of rosin or resinous vapor, passing to receiver number two. These receivers are kept at so low a temperature as to condense the whole of the products from the said still.

Various gases may be employed, instead of the steam, with very similar effect; but we do not find the results equal to those obtained by steam.

The solid contents of the receivers during the distillation, as conducted by either of the above-mentioned processes, are found to vary in their characteristics at different stages of the process. At three stages of the process we find this variation to be very marked, and we have accordingly distinguished the distillates as obtained during the three periods as follows: That obtained during the first stage of the distillation, and which amounts to about one-fourth of the original matter placed in the still, we call "alpha-rosin" or "alpha-resin;" that which is obtained after the removal of the said alpha-rosin or alpha-resin, and during the second stage of the said process, and which also amounts to one-fourth of the said original matter, we call "beta-rosin" or "beta-resin;" that obtained in the said receiver on the re-

moval of the said beta-rosin or beta-resin, and during the third stage of the said process, and which forms the remainder of the said original matter, we call "gamma-rosin" or "gamma-resin." These three several substances present the characteristics of resins, but clarified and to a great extent deprived of color. They are, either separately or in combination, applicable to and useful in the manufacture of several important articles of use—such as soap, size, caudles, paper-varnish, and japan, and for distilling to produce resin-oils.

Having thus described the nature of our invention and the best means with which we are acquainted of performing the same, we would have it understood that we are aware that stills and steam-worms capable of distributing small jets of steam have been before used in a somewhat similar way for the treatment of oils and fatty matters, and for improving the quality of resin-oil obtained from substances similar to those used by us in the processes hereinbefore described; but such a process has never, so far as we can ascertain, been applied to any such substances as are proposed to be operated upon by our processes for the purposes of obtaining the resinous and solid products above specified as the result of our said processes.

We therefore claim as our invention or discovery and desire to have secured to us by Letters Patent—

The new articles of commerce hereinabove specified as produced by the processes hereinabove mentioned, or by any similar mode or process, said articles or products not having been hitherto known in commerce or used in the arts.

In witness whereof we have hereunto subscribed our names.

EDWARD HUNT.

HENRY DAVIS POCHIN.

Witnesses:

THOS. BRITTAU,

SAMUEL LEE,

Clerks with Mr. Binney, Solicitor, 40 Cross Street, Manchester.